

# UNITED STATES PATENT OFFICE.

THOMAS H. VERHAVE, OF THE HAGUE, NETHERLANDS.

## MANUFACTURE OF THREADS FROM VISCOSE.

1,280,338.

Specification of Letters Patent.

Patented Oct. 1, 1918.

No Drawing.

Application filed February 23, 1915. Serial No. 9,916.

To all whom it may concern:

Be it known that I, THOMAS HERMANUS VERHAVE, subject of the Queen of the Netherlands, residing at The Hague, Adelheidstraat 99, Netherlands, have invented a new and useful Manufacture of Threads from Viscose; and I do hereby declare the following to be a full, clear, and exact description of the same.

10 It is known that good shiny artificial silk threads can be obtained from viscose only after the latter has been standing some time. The molecules of cellulose xanthogenate then coalesce, a process which is 15 known as the ripening of the viscose. The more the viscose is ripened or seasoned either by a long ripening process, or by subjecting it to a high temperature, the more satisfactory is the precipitation. If ripened 20 sufficiently, the precipitation takes place spontaneously.

It has been found that viscose which has been kept for 7 to 8 days at a temperature of 16°, is the most suitable for spinning. 25 Such viscose requires for its precipitation only a very small quantity of free hydrogen ions, which has the advantage that the newly formed thread, when escaping from the spinning nozzle, is not damaged by an 30 excessive concentration of acid during its travel through the spinning bath. If, however the viscose contains a large quantity of 35 free soda-lye in order to form a sufficiently thin fluid, an alkaline reaction of the spinning bath would soon take place. A good 40 spinning bath must therefore have a low concentration of hydrogen ions. This concentration must however remain constant and therefore it must be automatically renewed as neutralization is effected by the hydroxyl ions of the viscose.

This result can be obtained in various ways, for instance by dissolving a weak acid in a solvent in which a strong dissociation taken place, for instance in water; 45 or by dissolving a strong acid in an organic liquid which has a small ionizing action; or finally by dissolving a strong acid in a medium having a good ionizing action and 50 by restraining the ionizing of the acid which takes place according to the known formula of equilibrium. For sulfuric acid this formula is



55 In order to restrain the ionizing, therefore, it is necessary to add a larger quantity

of  $\text{SO}_4^-$  ions to the solution of sulfuric acid, or in other words it is necessary to add a substance which in an aqueous liquid produces an ample quantity of  $\text{SO}_4^-$  ions, but no  $\text{H}^-$  ions, that is to say a sulfate. This possibility is however precluded by the limited solubility of the said salts. Thus for instance the spinning bath described in 60 German Patent No. 187947, with a viscose of the degree of ripeness described, produces a dull weak thread, which moreover is referred to in German Patent No. 240846, lines 20 to 22, and in other literature. This 65 is due to the quantity of the existing  $\text{SO}_4^-$  ions being still insufficient, compared to the proportion of hydrogen ions. In order to restrain sufficiently the ionizing of the acid, still more sodium sulfate should be dissolved, which however is not possible owing 70 to the limited solubility of sodium sulfate. 75

According to this invention, this disadvantage is obviated by dissolving in the liquid an additional quantity of sulfate, in 80 order to increase sufficiently the concentration of the  $\text{SO}_4^-$  ions. In the case of a proportion of about 10% of sulfuric acid, the concentration should be at least 3 gram-molecules per kilogram of the spinning bath, 85 that is to say 3 molecules of  $\text{SO}_4^-$  ions should be present to each two molecules of hydrogen ions. In the case of a modification of 90 the proportion of acid (which should be at least 7% in order to insure reliable precipitation of the cellulose) there should be at least 3 mol.  $\text{SO}_4^-$  ions for each 2 mol.  $\text{H}^-$  ions.

In the spinning bath described in German Patent No. 187947 there are only 3.3 molecules of  $\text{SO}_4^-$  ions to each 3 molecules of  $\text{H}^-$  ions, and the same conditions are found in the process described in the German Patents Nos. 240846 and 260479.

A suitable composition of a spinning bath according to this invention, for a viscose of 100 the above mentioned degree of ripeness is for instance as follows:

16 parts  $\text{Na}_2\text{SO}_4$ ,  
30 parts crystallized magnesium sulfate 105  
 $\text{MgSO}_4 \cdot 7\text{H}_2\text{O}$ ,  
9 parts  $\text{H}_2\text{SO}_4$ ,  
45 parts water.

The salts could be however replaced by other easily soluble sulfates. 110

What I claim is:

1. In the manufacture of threads from viscose, the introduction of the latter into a spinning bath which contains two easily-

soluble sulfates added in such quantity to an aqueous solution of sulfuric acid of not materially less than 7 per-cent, that the resultant solution contains at least 3 mol. 5  $\text{SO}_4$  ions to each 2 mol. H-ions.

2. In the manufacture of threads from viscose, the introduction of the latter into a spinning bath which contains a plurality of easily-soluble sulfates added in such 10 quantity to an aqueous solution of sulfuric

acid of not materially less than 7 per-cent, that the resultant solution contains at least 3 mol.  $\text{SO}_4$  ions to each 2 mol. H-ions.

In testimony whereof I have signed my name to this specification in the presence of 15 two subscribing witnesses.

THOMAS H. VERHAVE.

Witnesses:

NICOLAAS J. C. HOLDEMAN,  
KUUN WIJNBRAUS.